

April 17, 1928.

1,666,214

J. S. LITTLE

METHOD OF COATING CORES

Filed April 17, 1926

3 Sheets-Sheet 1

Fig. 1.



Fig. 3.



Inventor  
John Shirley Little  
by *Macfarlan* Att'y.

April 17, 1928.

1,666,214

J. S. LITTLE

## METHOD OF COATING CORES

Filed April 17, 1926

3 Sheets-Sheet 2



Inventor  
John Shirley Little  
by McFettrick Att'y.

April 17, 1928.

1,666,214

J. S. LITTLE

## METHOD OF COATING CORES

Filed April 17, 1926

3 Sheets-Sheet 3



Fig. 6.



Fig. 8.  
69

Fig. 9.



Fig. 10.



Fig. II.



Fig. 7.



Inventor  
John Shirley Little  
By Habermann  
Atty.

## UNITED STATES PATENT OFFICE.

JOHN SHIRLEY LITTLE, OF CHICAGO, ILLINOIS, ASSIGNOR TO WESTERN ELECTRIC COMPANY, INCORPORATED, OF NEW YORK, N. Y., A CORPORATION OF NEW YORK.

## METHOD OF COATING CORES.

Application filed April 17, 1926. Serial No. 102,714.

This invention relates to a method of coating cores, and more particularly to a method of coating a core in strand form with pulpous material.

5 The object of the invention is to facilitate the application of pulpous material to a core in strand form and the formation of the pulpous material thereon to constitute a substantially uniform and uninterrupted 10 coating therefor.

Briefly stated, the improved method consists in bringing the core into intimate relation with a liquid containing pulp and a comparatively small quantity of soap in such 15 manner that pulp is applied to the core and caused to cling thereto. Excess moisture is then removed from the pulpous material applied to the core and the pulpous material is formed into a substantially uniform and 20 uninterrupted coating for the core which is subsequently dried by being subjected to circulating air of predetermined relative humidity and temperature.

The present method may be employed to 25 advantage for insulating electrical conductors, but it is to be understood that it is capable of other applications and should be limited only in so far as defined in the appended claims. Where the method is used 30 for insulating electrical conductors, manila, wood, r. gs, cotton, esparto, jute, hemp and asbestos, pulp may be employed as the coating material, but other materials than those specified may be used without departing 35 from the spirit and scope of the invention which contemplates in its broadest aspect the coating of a core in strand form with pulpous material in the presence of soap.

The term "core in strand form" as used 40 in the specification and appended claims refers to a core having a configuration resembling a fiber, hair, filament, string, small core or the like, or in the nature of a rope consisting of fibers, yarns and wire twisted 45 together.

It is believed that the improved method will be clearly understood from the following description of an apparatus by which the method may be practiced and the accompanying drawings, in which:

Figs. 1 and 2 are complementary parts of a plan elevation of an apparatus by which the improved method may be practiced;

Figs. 3 and 4 are complementary parts of

a longitudinal section through the apparatus 55 shown in Figs. 1 and 2;

Fig. 5 is a plan view of a portion of the apparatus shown in Figs. 1 to 4 inclusive, this portion of the apparatus being adapted to subject a plurality of cores in strand 60 form to a liquid containing pulp and a comparatively small quantity of soap;

Fig. 6 is a section taken on the line 6—6 of Fig. 5;

Fig. 7 is a section taken on line 7—7 of 65 Fig. 6, and

Figs. 8 to 11 inclusive are enlarged transverse sections which progressively illustrate the manner in which the apparatus shown in 70 Figs. 1 to 7, inclusive, coat a core with pulpous material.

The apparatus illustrated in the drawings is adapted to coat a plurality of cores in strand form simultaneously, the cores being subjected to a liquid containing pulp and a comparatively small quantity of soap in 75 such manner that pulp is deposited on the cores uniformly. Excess moisture is then squeezed from the pulpous material applied to the cores and the pulpous material is formed into a uniform and uninterrupted 80 coating which is dried in air of predetermined relative humidity and temperature.

The portion of the apparatus which applies the pulpous material to the cores and removes the excess moisture therefrom is termed the "wet end" of the apparatus and is designated in the drawings by the reference character 15. The "wet end" comprises a drum 16 which is partly submerged in a 85 liquid containing pulp held in a tank 17. As shown in Figs. 5 to 7 inclusive, the drum 16 comprises a plurality of spiders 18 rigidly secured to a shaft 19 which is rotatably journaled in a plurality of bearings 20 mounted upon hollow side walls 32 of the tank 17. A 90 plurality of bars 22 secured to the spider 18 form a support for a helical member 23 which is formed of a rod wound around the bars. The helical member 23 supports a 95 coarse mesh screen 24 which in turn supports a fine mesh screen 25, the fine mesh screen 25 being covered by a plurality of rings or dams 26 of some waterproof material, such as okonite. The bars 22, the 100 helical member 23, the screens 24 and 25, and the dams 26 together form a cylindrical wall for the drum 16, the dams 26 being 105

spaced from each other to provide a plurality of annular passages 27 through which liquid may flow from the tank 17 into the drum 16.

Each end of the drum 16 is provided with an annular member 30 disposed concentrically with respect to the axis of the shaft 19. The outer end of each annular member is disposed in close proximity with an annular flange 31 formed in each side wall 32 of the tank 17. Each side wall 32 has a chamber 33 which communicates with the interior of the drum 16 through an aperture 34 formed in the side wall, and through the annular flange 31 and the adjacent annular member 30. Formed in the bottom of the tank 17 between the chambers 33 is a passage 35 through which the liquid may flow from the left hand chamber 33 to the right hand chamber 33 and thence through a pipe 38 communicating with the right hand chamber 33. It is obvious that if liquid containing pulp is introduced into the tank 17 the free liquid will flow through the annular passages 27 into the drum 16 and then into the chambers 33 from which it may be drawn by way of the pipe 38.

The liquid containing pulp is supplied to the tank 17 from a mixing vat (not shown) through a pipe 48 (Fig. 6). In practice, pulpos material suitable for the manufacture of paper may be employed. A comparatively small amount of soap is introduced into the pulpos material, preferably before it enters the tank 17. The liquid soap may be supplied from a suitable receptacle 40 communicating with the pipe 48 through a pipe 41, the pipe 41 being provided with a suitable valve 42 for controlling the amount of soap introduced into the pulpos material as it passes through the pipe 48 into the tank 17. The receptacle 40 may be supported by a plurality of brackets 43 secured to a wall 49 of the tank 17. The pipe 48 discharges into a space or compartment formed at one end of the tank 17 by the wall 49 and a second wall 50 suitably spaced therefrom.

The liquid containing pulp is preferably introduced into the tank 17 under pressure by means (not shown) which insures a forced circulation of the pulpos material through the apparatus. A plurality of baffle plates 51 disposed between the walls 49 and 50 insure that the pulpos material and the soap will be thoroughly mixed before entering the tank proper by passing over the wall 50 which is of lesser height than the wall 49.

The means (not shown) for maintaining a circulation between the mixing vat (not shown) and the tank 17 may be adjusted to keep the pulp mixture at a predetermined level in the tank. The liquid in the drum 16 is maintained at a lower level than that of the pulp mixture in the tank. Should the level of the liquid within the drum 16 tend

to rise above a predetermined point, the excess liquid will flow over a plurality of vertically disposed gates 58 provided in the chambers 33. The gates 58 are slidably mounted in the chambers 33 and may be secured in adjusted positions by means of wing nuts 60 threaded upon bolts 61 projecting from the gates through slots 62 formed in the side walls 32 of the tank. Liquid flowing over the gates 58 is discharged from the apparatus through a plurality of drain pipes 64.

As shown in Figs. 2 and 4, the cores which are subjected to the liquid containing pulp are withdrawn from a plurality of supply reels 65 mounted upon a shaft 66 which is mounted in a plurality of brackets 67. The cores, which are indicated by the reference character 69, are trained over a plurality of sheaves 70 carried by a shaft 71 which is mounted in the side walls 32 of the tank 17. From the sheaves 70 the cores 69 are trained around the annular foraminous passages 27 of the drum 16, each core 69 being centrally disposed in one of the passages. The drum is rotated by the cores as they are drawn through the apparatus, a ribbon of moist pulpos material being formed in each passage 27 and attached to each core as it passes around the drum. The construction is such that a layer of pulp is strained onto the fine mesh 25 before the cores are brought into contact therewith. Then, after the cores contact the initial layers of pulp on the screen and the drum continues to revolve in the tank, an additional amount of pulp is deposited on each core and the screen. The pulpos material deposited upon the cores and the screen 25 adheres to the cores in the form of ribbons 73 as illustrated in Fig. 7. A woven belt 75 aids in freeing the pulp ribbons from the screen 25 when the cores leave the drum 16, the belt 75 being held into contact with the drum by a felt covered roller 76 rotatably mounted in a frame 77. The felt covered roller 76 coats with the belt 75 and the drum 16 to squeeze the excess liquid from the pulpos material adhering to the core, the core and its ribbon of pulpos material being advanced with the belt 75 and between it and a similar belt 79.

The presence of soap in the liquid containing pulp improves and facilitates the formation of the pulpos ribbons on the cores. Furthermore, it has been found in the practice of this invention that the addition of a small amount of soap to the pulpos material facilitates freeing the pulpos ribbons from the drum 16 by the belt 75.

The belt 75 is trained over a plurality of rubber covered rollers 80 and 81 and over a plurality of rolls 83, the rollers 80 and 81 and the rolls 83 being rotatably journaled in the frame 77. Means (not shown) is provided for driving the roller 80 and it drives

the belt 75 which in turn drives the belt 79, the belt 79 being held in contact with the belt 75 by means of a plurality of rubber covered rollers 85 and 86. The rubber covered rollers 81 and 86 coat with each other and with the belts 75 and 79 to squeeze excess moisture from the ribbons of pulpoous material adhering to the cores. The rollers 80 and 85 also function in this manner. The belts 75 and 10 79 are sufficiently porous to allow the liquid to escape therethrough. This construction is particularly advantageous in that the belts 75 and 79 prevent the cores from "whipping" as they travel from the squeezing rollers 15 81 and 86 to the squeezing rollers 80 and 85, it being obvious that "whipping" of the cores would be accompanied by displacement of the ribbons of pulpoous material relative to the cores. The belt 75 supports 20 the cores and the pulpoous ribbons as they are advanced from one pair of squeezing rollers to the other in such manner that the pulp ribbons will not dangle from the cores and lose the form which is imparted to them by 25 the felt roller 76 and the drum 16. Fig. 9 illustrates the form which is imparted to each ribbon of the pulpoous material by the felt covered roller 76 and the drum 16. The belts 75 and 79 also facilitate the task of 30 coating a plurality of cores simultaneously as the belts hold the cores to parallel paths as they are advanced from the squeezing rollers 81 and 86 to the squeezing rollers 80 and 85. This prevents the ribbons of pulp 35 from becoming entangled with each other. The ribbons of pulpoous material are sufficiently dry, when they leave the wet end 15, that the cores alone will support them.

A plurality of forming mechanisms 90 are 40 adapted to receive the cores 69 with the ribbons of pulpoous material when they are discharged from the wet end 15, a plurality of sheaves 95 being provided for guiding the cores to the forming mechanisms. The 45 forming mechanisms 90 may be of the type shown and described in the copending application of H. W. Jespersen, Serial No. 713,704, filed May 16, 1924, and are rotatably mounted in a hollow frame 91, means indicated at 92 being provided for rotating the 50 forming mechanisms. The forming mechanisms 90 are adapted to wrap each pulpoous ribbon around itself and around the core associated therewith to form a uniform coating for the core. The manner in which a 55 pulpoous ribbon is wrapped around itself and around a core is illustrated in Fig. 10, the fully formed coating being shown in Fig. 11.

The presence of soap in the liquid containing pulp materially minimizes any tendency of the forming mechanisms to strip the pulpoous ribbon from the core, thereby insuring a substantially uniform and uninterrupted coating throughout the length of the core. 65 Furthermore, it has been found in the prac-

tice of this invention that by the addition of a comparatively small amount of soap to the liquid containing pulp, the tendency of small portions of the pulpoous ribbon to become attached to the polishing blades of the forming mechanisms is minimized, thus decreasing the amount of attention the forming mechanisms require. 70

After leaving the forming mechanisms the coated cores are guided by a plurality of 75 sheaves 96 into a housing or compartment 100 wherein they are dried, a plurality of sheaves 101 being provided to guide them through a plurality of apertures 102 formed in one of the walls of the compartment. 80 The coated cores are trained over a plurality of sheaves 103 mounted in the compartment 100 and are discharged from the compartment through a plurality of apertures 105 formed in another wall thereof. Means indicated at 106 is provided for subjecting the pulpoous coatings on the cores to air of predetermined relative humidity and predetermined temperature. This means is described in detail in my Patent No. 1,615,393, dated 90 January 25, 1927, and since it forms no part of this invention no particular description thereof is given in this disclosure. After the coated cores pass from the compartment 100 they are guided by a plurality of sheaves 95 105 108 to a plurality of take-up spools 109 which are driven by any suitable means (not shown).

What is claimed is:

1. A method of coating a core in strand form consisting in subjecting the core to a liquid containing pulp in the presence of soap in such manner that pulp is applied thereto, and then forming the pulp around the core to constitute a coating conforming 100 with the core and retained on the core by a felting of the pulp fibers. 105

2. A method of coating a core in strand form consisting in applying pulp to the core in the presence of soap in such manner that a ribbon of pulp is attached to the core, and subsequently forming the pulpoous ribbon on the core to constitute a coating retained on the core by a felting of the pulp fibers. 110

3. A method of coating a core in strand form consisting in subjecting the core to a liquid containing pulp in the presence of soap in such manner that pulp is applied thereto, squeezing the pulp on the core to remove excess moisture therefrom and form 115 it into a ribbon, and then wrapping the pulpoous ribbon around itself and around the core to constitute a coating therefor. 120

4. A method of coating a core in strand form consisting in attaching a ribbon of wet 125 pulp in the presence of soap to the core, and then forming the pulpoous ribbon on the core to constitute a coating encircling the core and attached thereto by an intermingling of the pulp fibers. 130

5. A method of coating a core in strand form which consists in subjecting the core to a solution of pulpoous material including a liquid soap in such manner that a ribbon of wet pulp is caused to cling to the core, squeezing said pulpoous ribbon to remove excess moisture therefrom, and then forming said ribbon to constitute a coating having a curved outer surface and attached thereto by a felting of the pulp fibers.

6. The method of coating a core in strand form consisting in applying pulpoous material in the presence of soap to the core, and then forming the pulpoous material on the core to constitute a coating therefor.

7. A method of coating a core in strand form consisting in applying pulpoous material in the presence of soap to the core, and then forming the pulpoous material on the core to constitute a coating having a curved outer surface.

8. A method of coating a core in strand form consisting in applying a core to a liquid containing pulp and a relatively small percentage of soap in such manner that a ribbon of wet pulp is caused to cling to the core, squeezing said pulpoous ribbon to remove excess moisture therefrom, and subsequently wrapping the pulpoous ribbon around itself and around the core to constitute a coating conforming to the shape of the core and retained thereon by a felting of the pulp fibers.

9. A method of coating a core in strand form consisting in subjecting the core to a liquid containing pulp in the presence of soap in such manner that pulp is applied thereto, forming the pulp around the core to constitute a coating conforming with the core and retained thereon by a felting of the pulp fibers, and then subjecting the coated core to air of predetermined relative humidity and temperature.

10. A method of coating a core in strand form consisting in subjecting the core to a liquid containing pulp in the presence of soap in such manner that a ribbon of wet pulp is attached to the core, squeezing said pulpoous ribbon to remove excess moisture therefrom, forming the ribbon on the core to constitute a coating conforming to the shape of the core and attached thereto by a felting of the pulp fibers, and then drying the coated core in air of predetermined relative humidity and temperature.

11. A method of coating a core in strand form, which consists of adding a small quantity of soap to a liquid containing pulp, applying the slightly soaped pulp to the core, and forming the pulp around the core to constitute a uniform coating.

In witness whereof, I hereunto subscribe my name this 26th day of March, A. D. 1926.

JOHN SHIRLEY LITTLE.